

[54] **LOW POUR POINT GAS FUEL FROM WAXY CRUDES**

[76] Inventor: **William M. Sweeney**, Texaco Inc.  
P.O. Box 509, Bacon, N.Y. 12508

[22] Filed: **July 9, 1970**

[21] Appl. No.: **53,659**

**Related U.S. Application Data**

[63] Continuation-in-part of Ser. No. 881,358, Dec. 2, 1969, abandoned.

[52] **U.S. Cl.** ..... 44/62, 44/70

[51] **Int. Cl.** ..... C10I 1/18

[58] **Field of Search** ..... 44/62, 70, 80; 252/56; 208/15/17

[56] **References Cited**

**UNITED STATES PATENTS**

2,664,388 12/1953 Wintehalter ..... 208/15  
3,567,639 3/1971 Aaron et al. ..... 44/62

3,640,691 2/1972 Ilnyckyj et al. ..... 44/80

*Primary Examiner*—Daniel E. Wyman

*Assistant Examiner*—Mrs. Y. H. Smith

*Attorney, Agent, or Firm*—T. H. Whaley; C. G. Ries

[57] **ABSTRACT**

A low pour point gas turbine fuel is prepared from a waxy crude by blending a 650°-750°F distillate fraction from a crude oil with a minor amount of a 350°-650°F fraction of a middle distillate and from 0.05 to 0.5% by weight of an oil-soluble ethylene-vinyl fatty acid ester copolymer in which the fatty acid component of the ester has a carbon content of from about 2 to about 6; the copolymer having a molecular weight between about 17,000 and 29,000, and a vinyl fatty acid ester content of from about 27 to about 42. The melt index of the copolymer ranges from 7 to 465.

**4 Claims, 1 Drawing Figure**



PATENTED JAN 28 1975

3,862,825



## LOW POUR POINT GAS FUEL FROM WAXY CRUDES

This application is a continuation-in-part of Ser. No. 881,358 filed Dec. 2, 1969, now abandoned.

### BACKGROUND OF THE INVENTION

This invention is concerned with means for providing a turbine fuel composition at a reduced cost. More particularly, the invention is concerned with a turbine fuel composition containing a major amount of cheaper higher boiling constituents and a minor amount of more expensive middle distillate, this fuel still meeting pour point specifications owing to the incorporation therein of certain high molecular weight ethylene-vinyl fatty acid ester copolymers.

As is well known, gas oils distillates boiling at 650°-750°F. contain quantities of wax which render them viscous and give unacceptably high pour points. These oils behave as non-Newtonian liquids at low temperatures: exhibit variable solidifying temperature and peculiar hysteresis phenomena — all of which render them difficult to use as fuel.

One approach used in converting these oils has been to subject them to fairly lengthy dewaxing procedures. This, however, is an expensive procedure.

Another approach which has been used to bring the viscosity of "crude" gas oils to suitable levels has been to dilute or "cut" them with a major amount of lighter distillate oils but this is an expensive procedure because of the considerably higher cost of the distillate oils relative to the higher boiling oils. Generally, the ratio of distillate to higher boiling gas oil used has been 9 to 1. The distillate can be sold directly as a diesel fuel and as such is valuable and in short supply.

A number of additives have been suggested and tried with success in lubricating oils and in so-called middle distillates in order to tie in the wax therein and improve flow at low temperatures. Such additives consist either of compounds formed by alkylating benzene or naphthalene derivatives or of copolymers of ethylene-vinyl fatty acid ester of a molecular weight up to 3,000 and containing from 15 to 25% by weight of the vinyl fatty acid ester. These additives are not, however, effective in depressing the pour point of crude turbine fuel oils.

It is therefore the main object of the present invention to provide a fuel composition based on crude oil which will be free of the above mentioned prior art limitations.

An equally important object of this invention is to provide a turbine fuel oil composition having improved pour point characteristics by incorporating therein a minor amount of distillate oil and a small amount of certain ethylene-vinyl fatty acid ester copolymers.

Other objects of this invention will in part be obvious and in part hereinafter pointed out.

The turbine fuel oil of the invention comprises from 55 to 90% by weight of crude gas oil fraction boiling at about 650°-750°F. and a pour point depressant additive including from 10 to 45% by weight of middle distillate oils boiling from 350° to 650° and from 0.01 to about 0.5% by weight of ethylene-vinyl fatty acid ester copolymers having a molecular weight of about 17,000 to 25,000 with a vinyl fatty acid ester (C<sub>2</sub>-C<sub>6</sub>) content of about 24 to 42%, and a melt index of from 7 to 465.

The preferred additives contain 27 to 42% ethylene-vinyl acetate copolymer having a melt index of 22 to 465 and a molecular weight ranging from about 18,000 to 21,000.

- 5 The characterization of the "Elvax" copolymers is given in Table III below. These can be added in the form of a hydrocarbon solution concentrate in, for example, toluene, in the 350°-650°F. middle distillate fraction or even in the middle distillate-gas oil mixture.
- 10 The ethylene-vinyl fatty acid ester additives are then added to the gas oil and mixed with the middle distillate in an amount in the range of 0.01% to about 0.05% by weight of the composition.
- 15 The additives may be prepared by any convenient process, such as that of U.S. Pat. No. 3,215,678, by a free radical-initiated polymerization of ethylene and a vinyl ester of a lower saturated monobasic aliphatic carboxylic acid. The effectiveness of the additives according to the invention is demonstrated by the following examples in which the pour points given were obtained by ASTM Method D-97-47.

### EXAMPLE I

There was charged to a still Mata crude oil from Guatemala which had the following characterization:

|    |                                                                                  |       |
|----|----------------------------------------------------------------------------------|-------|
|    | % Wax St 265 — dissolve in MIB ketone — cool 0°F.<br>filter and weight wax, etc. | 2.03  |
|    | Gravity°API                                                                      | 30.06 |
|    | % Sulfur, X-ray                                                                  | 0.86  |
|    | Wt. % Ash                                                                        | 0.002 |
| 30 | Kin. Viscosity, cs at 100°F.                                                     | 7.52  |
|    | at 150°F.                                                                        | 3.79  |
|    | Carbon residue, wt. %                                                            | 3.89  |
|    | Flash pt, PM, °F.                                                                | 58.4  |
|    | Basic Nitrogen, ppm                                                              | 3.93  |
| 35 | Total Nitrogen, ppm                                                              | 1573  |
|    | Pour Point, °F.                                                                  | -15   |

The percent of wax was determined by dissolving a sample of the oil in methyl isobutyl ketone, cooling the resulting solution to 0°F., filtering off the wax and weighing it. The fraction boiling from 350°-650°F. (atmospheric) was obtained in 34% yield and had a pour point of -5°F. The fraction boiling from 650°-750°F. was obtained in 11.3% yield and had a pour point of +100°F. Blends of the two oils in different proportions were prepared and their kinematic viscosities (cs at 100°F.) and their pour points were determined. The Table I below shows the values obtained.

TABLE I

|    | Wt. % of 350-650°F. cut | Wt. % of 650-750°F. cut | Kin. Vis. | Pour Point (°F.) |
|----|-------------------------|-------------------------|-----------|------------------|
|    | 0                       | 100                     | 13.69     | + 65             |
|    | 10                      | 90                      | 10.63     | + 55             |
|    | 25                      | 75                      | 7.83      | + 55             |
| 55 | 40                      | 60                      | 5.45      | + 50             |
|    | 100                     | 0                       | 2.43      | - 5              |

### EXAMPLE II

A 30% solution of Zetafax 1575 (an ethylene-vinyl acetate copolymer containing about 27% by weight of vinyl acetate and having a molecular weight of 20,000 and a Melt Index of 12-18) was prepared by dissolving by heating in toluene on a steam plate 0.1% by weight of the copolymer and incorporated in a mixture of 90% gas oil (650°-750°F.) and 10% distillate (350°-650°F.)

and pour point, cloud point and viscosity determinations were made on the resulting mixture as well as on the pure mixture and the gas oil. The results obtained are tabulated below:

TABLE II

| Fuel Blend                                | Cloud Point | Pour Point<br>°F.    | Viscosity                             |
|-------------------------------------------|-------------|----------------------|---------------------------------------|
| 100% gas oil<br>(650-750°F.)              | —           | 65                   | 14.2                                  |
| 90% gas oil<br>(650-750°F.)               | 62          | 55                   | 10.6                                  |
| + 10% distillate<br>(350-650°F.)<br>alone |             |                      |                                       |
| + 0.1% additive<br>above mixture          | 64          | -20/-35 <sup>a</sup> |                                       |
| GE 1 410970<br>Specifications             | —           | 0 (Max)              | about 10cs<br>(Max at the<br>nozzles) |

<sup>a</sup> Maximum pour point.

In the above tests, the pour point is determined by the ASTM D-97 method. The maximum pour is determined by reheating the above sample to 220°F. and then storing at 0°F. or at a temperature below the maximum pour, whichever is lower, for at least 12 hours. The sample is then removed from cold storage, placed in a 115°F. bath till warm and the pour point is determined. This maximum pour point determination yields a value for the pour point above which a given sample will not revert under prolonged storage or when exposed to a cyclic temperature environment.

Comparison of the data presented in Tables I and II shows immediately the advantage of the invention. It will be seen in particular that by using the additive of the invention, pour specifications can be met using 98% of the crude oil with only 10% of the more valuable 350°-650°F. middle distillate. On the other hand, without the additive, 95% of the middle distillate would be required with 5% of the crude gas oil (650°-750°F.) to achieve the desired pour point.

In other examples of the practice of the invention 0.05% of various Elvax copolymers were blended with 50 100% vacuum gas oil (Mata) and the pour points of each blend as well as of the additive-free oil were determined. The results thus obtained are tabulated below in Table III. The best pour point reduction is obtained with the copolymer which has from 27-29% of vinyl acetate and a melt index of 340-470 g/10 mm.

TABLE III

Pour Points of mixtures of various ELVAX Copolymers in 100% Vacuum Gas Oil (MATA) at 0.05% Concentration

| ELVAX | Pour Point, % | % Vinyl Acetate<br>in Copolymer | Melt Index* |
|-------|---------------|---------------------------------|-------------|
| 40    | +45           | 39-42                           | 45-70       |
| 150   | +45           | 32-34                           | 22-28       |
| 210   | +25           | 27-29                           | 335-465     |
| 220   | +45           | 27-29                           | 125-175     |
| 240   | +50           | 27-29                           | 22-28       |
| 250   | +55           | 27-Q9                           | 12-18       |
| 260   | +60           | 27-29                           | 5-7         |
| 310   | +55           | 24-Q6                           | 335-465     |
| 350   | +55           | 24-26                           | 16-22       |
| 360   | +60           | 24-26                           | 1.6-2.4     |
| 410   | +55           | 17-19                           | 430-580     |
| 460   | +65           | 17-19                           | 2.1-2.9     |
| None  | +65           | —                               | —           |

\* in g/10 min. as determined by ASTM D 1328 modified.

The results obtained by the invention are graphically illustrated in the accompanying figure. In the figure the pour points of various blends of vacuum gas oil with middle distillates are plotted (top line). The plot of these with 0.125 and 0.1% of Elvax 210 is also given as well as that of 0.05% of the same additive in 100% vacuum gas oil.

It will be evident to those skilled in this art that the pour point depressants of this invention may be used along with other additives usually found in fuel oils of the character described. Such other additives will include rust inhibitors, anti-emulsifying agents, anti-static agents, anti-oxidants and the like.

I claim:

1. A fuel oil composition having improved pour point characteristics consisting of from 55 to 90 percent by weight of a gas oil boiling at about 650° to about 750°F and an additive consisting of from 10 to 45 percent by weight of a middle distillate boiling from about 350° to about 650°F, with an effective pour point depressant amount of an oil soluble ethylenevinyl fatty acid ester copolymer in which the fatty acid component of the ester has a carbon content of from about 2 to about 6, said copolymer having a molecular weight of from about 17,000 to about 29,000, a vinyl fatty acid ester content of from about 24 to about 42% and a melt index of 7 to 465.

2. A composition according to claim 1 wherein said vinyl ester is vinyl acetate.

3. A composition according to claim 1 wherein said copolymer is present in a concentration from about 0.01 to about 0.5% by weight of said composition.

4. The composition according to claim 1 wherein said copolymer is an ethylene-vinyl acetate copolymer having a molecular weight ranging from 18,000 to 21,000, an ethylene-vinyl acetate content ranging from about 27 to 42% and a melt index of 7 to 465.

\* \* \* \* \*